



US005411604A

**United States Patent** [19]

Inokuti et al.

[11] Patent Number: **5,411,604**[45] Date of Patent: **May 2, 1995**

[54] **METHOD OF PRODUCING LOW IRON LOSS, LOW-NOISE GRAIN-ORIENTED SILICON STEEL SHEET, AND LOW-NOISE STACKED TRANSFORMER**

[75] Inventors: **Yukio Inokuti, Kazuhiro Suzuki**, both of Chiba; **Eiji Hina**, Okayama, all of Japan

[73] Assignee: **Kawasaki Steel Corporation**, Japan

[21] Appl. No.: **8,531**

[22] Filed: **Jan. 26, 1993**

[30] **Foreign Application Priority Data**

May 29, 1992 [JP] Japan ..... 4-139047

[51] Int. Cl.<sup>6</sup> ..... **H01F 30/06**

[52] U.S. Cl. ..... **148/112; 219/121.17;**  
219/121.35

[58] **Field of Search** ..... 148/111, 112, 113;  
219/121.34, 121.25, 121.17, 121.14, 121.20,  
121.12

[56] **References Cited**

**U.S. PATENT DOCUMENTS**

3,076,160 1/1963 Daniels ..... 148/111  
4,915,750 4/1990 Salsgiver et al. ..... 148/112  
4,919,733 4/1990 Salsgiver et al. ..... 148/113  
5,146,063 9/1992 Inokuti ..... 219/121.35

*Primary Examiner*—George Wyszomierski  
*Attorney, Agent, or Firm*—Austin R. Miller

[57]

**ABSTRACT**

A grain oriented silicon steel sheet which exhibits reduced iron loss and which contributes excellent noise characteristics when used as a material of a stacked transformer. The sheet is produced by applying electron beam irradiation a finish-annealed grain oriented silicon steel sheet, along scan paths which cross the rolling direction at a scanning speed  $v$ (cm/s) and a spacing  $L$ (cm) in the rolling direction, with an electron beam of a beam diameter  $d$  (cm) generated by a current  $I_b$  (mA) and acceleration voltage  $V_k$  (kV);

wherein the surface energy density  $\alpha$  (J/cm<sup>2</sup>) on the surface of said steel sheet as determined by the following formula (1) is about 0.16 J/cm<sup>2</sup> or more, and said surface energy density  $\alpha$  (J/cm<sup>2</sup>) and the surface energy density  $\beta$  (J/cm<sup>2</sup>) on the scan paths meet the approximate condition of the following formula (3):

$$\alpha = (V_k I_b) / (L \cdot v) \quad (1)$$

$$\beta = (V_k I_b) / (d \cdot v) \quad (2)$$

$$0.6 - 0.06 \beta \leq \alpha \leq 0.90 - 0.08 \beta \quad (3)$$

Disclosed also is a stacked transformer produced from this grain oriented silicon steel sheet.

**8 Claims, 4 Drawing Sheets**

| dBi - dB <sub>i</sub> (dB) |                        |
|----------------------------|------------------------|
| ●                          | 5 OR MORE              |
| ○                          | 2 OR MORE, LESS THAN 5 |
| ◎                          | LESS THAN 2            |



FIG. 1



FIG. 2

|   | W17/50 (W/kg)                |
|---|------------------------------|
| • | 0.83 OR MORE                 |
| ○ | 0.78 OR MORE, LESS THAN 0.83 |
| ◎ | LESS THAN 0.78               |



FIG. 3

|   | $dB_i - dB'_i$ (dB)    |
|---|------------------------|
| • | 5 OR MORE              |
| ○ | 2 OR MORE, LESS THAN 5 |
| ◎ | LESS THAN 2            |



FIG. 4



**METHOD OF PRODUCING LOW IRON LOSS,  
LOW-NOISE GRAIN-ORIENTED SILICON STEEL  
SHEET, AND LOW-NOISE STACKED  
TRANSFORMER**

**BACKGROUND OF THE INVENTION**

**1. Field of the Invention**

This invention relates to electron beam irradiation for producing a reduced iron loss grain oriented silicon steel sheet which generates low noise when used in a stacked transformer. More particularly, this invention relates to a method of producing a grain oriented silicon steel sheet for use in a stacked transformer, where it achieves both reduced iron loss and reduced noise. This invention also relates to a stacked transformer comprising such grain oriented silicon steel sheets, which achieves significantly reduced noise generation in operation.

Grain oriented silicon steel sheets are used mainly as the core materials of electrical components such as transformers or the like. In general, grain oriented silicon steel sheets are required to have such magnetic characteristics that the magnetic flux density (represented by  $B_s$ ) is high and that the iron loss (represented by  $W_{17/50}$ ) is low. It is also required that the surfaces of the steel sheet have insulating films with excellent surfaces.

The energy crisis that the world now faces requires reduction of losses of electrical power. This has given rise to a strong demand for grain oriented silicon steel sheets having reduced iron loss.

**2. Description of the Related Art**

Grain oriented silicon steel sheets have undergone various treatments for improving magnetic characteristics. For instance, treatment has been conducted to attain a high degree of concentration of the secondary recrystallization grains in the Goss orientation. It has also been attempted to form, on a forsterite film formed on the surface of the steel sheet, an insulating film having a small thermal expansion coefficient so as to impart a tensile force to the steel sheet. Thus, grain oriented silicon steel sheets have been produced through complicated and diversified processes which require very strict controls.

Among these treatments, one major technique for reducing iron loss of grain oriented steel sheet has been the improvement of the aggregation structure of Goss orientation secondary recrystallization grains.

Hitherto, as a method for controlling the secondary recrystallization grains, preferential growth of Goss orientation secondary recrystallization grains has been obtained by using primary recrystallization grain growth inhibiting agents such as AlN, MnS and MnSe, known as "inhibitors".

In recent years various techniques other than metallurgical measures have been developed for controlling secondary recrystallization grains for reducing iron loss. For instance, techniques for reducing iron loss by irradiation with laser beams have been proposed in IRON AND STEELS, by Tadashi Ichiyama 69(1983), P895, Japanese Patent Publication No. 57-2252, Japanese Patent Publication No. 57-53419, Japanese Patent Publication No. 58-26405 and Japanese Patent Publication No. 58-26406. Methods also have been proposed which employ plasma irradiation as disclosed, for example, in Japanese Patent Laid-Open No. 62-96617, Japanese Patent Laid-Open 62-151511, Japanese Patent

Laid-Open No. 62-151516 and Japanese Patent Laid-Open No. 62-151517. In these methods local treatment is introduced into the steel sheet by irradiation of the steel sheet surface by laser beam or plasma, so as to refine the magnetic domains, thereby reducing iron loss.

These methods relying upon irradiation with laser beam or plasma, however, inevitably raise the cost of reducing iron loss, because the energy efficiency is as low as 5 to 20%.

Under these circumstances we have proposed a method in which an electron beam generated by electric power of high voltage and low current is locally and intermittently applied along the widthwise direction which intersects the rolling direction of the sheet, so as to forcibly introduce a coating film into the matrix iron. Such a method is disclosed, for example, in Japanese Patent Laid-Open No. 63-186826, Japanese Patent Laid-Open No. 2-118022 and Japanese Patent Laid-Open No. 2-277780.

This method exhibits very high energy efficiency, as well as high scanning speed, thus offering remarkably improved production efficiency as compared to known methods for refining magnetic domains.

The methods disclosed in our above-mentioned Japanese Patent Laid-Open specifications are directed to production of grain oriented silicon steel sheet for use as a material for a wound core transformer. In the production of a core of this kind, the wound core formed from a grain oriented steel sheet is subjected to stress-relieving annealing. Therefore, no substantial noise tends to be generated in the wound core transformer during operation of the transformer.

In contrast, a stacked transformer of that kind generates a high level of noise, requiring strong measures to be taken for reducing the noise.

In particular, the grain oriented steel sheets produced by the method proposed in the aforementioned Japanese Patent Laid-Open specification cannot be practically used in stacked transformers, due to high levels of noise.

On the other hand, U.S. Pat. No. 4,919,733 discloses a method for refining magnetic domains by irradiation with electron beams, wherein the surface energy density on the electron beam scan line is set to a level not lower than  $60 \text{ J/in}^2$  ( $9.3 \text{ J/cm}^2$ ). More specifically, Example 1 of this Patent shows that an electron beam treatment reduced the core loss at 1.7 T by about 10% when the treatment was conducted under the following conditions:

Beam acceleration voltage: 150 kV  
Beam current: 0.75 mA  
Scanning speed: 100 in/sec (254 cm/sec)  
Beam diameter: 5 mil (0.013 mm)

Irradiation line spacing: 6 mm.  
Steel sheets which have undergone this electron beam treatment, however, exhibit inferior noise characteristics when employed in a stacked transformer, as compared with steel sheets which have not undergone such electron beam treatment. In particular, the noise characteristics are extremely poor during operation of the transformer after the electron beam treatment has been conducted under the conditions mentioned above, as compared with sheets which have not undergone such treatment.

U.S. Pat. No. 4,915,750 proposes a method of producing a grain oriented silicon steel sheet for use as a material of a wound core transformer, employing refining of

magnetic domains by irradiation with an electron beam. This method is directed only to the production of a wound core transformer as distinguished from a stacked transformer to which the present invention pertains and which suffers from the noise problem.

#### SUMMARY OF THE INVENTION

Accordingly, an object of the present invention is to provide a method for stably producing a grain oriented steel sheet of high quality which exhibits not only reduced core loss but also significantly reduced noise when used in a stacked transformer.

It is also an object of the present invention to provide a stacked transformer having improved noise characteristics.

To these ends, according to one aspect of the present invention, we have created a method of producing a grain oriented silicon steel sheet which exhibits reduced iron loss and which, when used as a material of a stacked transformer, achieves sharply reduced noise characteristics.

The method of this invention is advantageously performed by preparing a finish-annealed grain oriented silicon steel sheet, irradiating the surface of the grain oriented silicon steel sheet along scan paths which cross the rolling direction of the steel sheet at a scanning speed  $v$  (cm/s) and a spacing  $L$  (cm) in the direction of rolling, such irradiation being performed with an electron beam of a beam diameter  $d$  (cm) generated by a current  $I_b$  (mA) and an acceleration voltage  $V_k$  (kV) and wherein the surface energy density  $\alpha$  ( $J/cm^2$ ) on the surface of said steel sheet is controlled as determined by the following formula (1) to about  $0.16 J/cm^2$  or more, and said surface energy density  $\alpha$  ( $J/cm^2$ ) and the surface energy density  $\beta$  ( $J/cm^2$ ) on the scan paths meet approximately the condition of the following formula (3):

$$\alpha = (V_k \cdot I_b) / (L \cdot v) \quad (1)$$

$$\beta = (V_k \cdot I_b) / (d \cdot v) \quad (2)$$

$$0.6 - 0.06\beta \leq \alpha \leq 0.90 - 0.08\beta \quad (3)$$

According to another aspect of this invention we have provided a low-noise stacked transformer produced in accordance with the method of the present invention.

#### BRIEF DESCRIPTION OF THE DRAWING

FIG. 1 is a diagram of an electron beam apparatus 50 which may be employed in the method of this invention.

FIGS. 2 and 3 are graphs indicating test results obtained in the testing of the invention, and

FIG. 4 is a diagram of another electron beam irradiating apparatus in accordance with the invention.

#### DETAILED DESCRIPTION OF THE INVENTION

A detailed description will now be given of an experiment, with reference to FIG. 1 which shows an electron beam irradiation apparatus employed in the experiment. The experiment is intended to be illustrative but not to limit the scope of the invention, which is defined in the appended claims.

Referring to FIG. 1, the electron beam irradiation apparatus has a vacuum chamber 1 in which vacuum is maintained by operation of a vacuum pump 2. Numeral

3 designates a grain oriented silicon steel sheet. The apparatus also has an electron beam gun 4 and a graphite roller 5. Numeral 6 denotes an electron beam emitted from the electron beam gun 4. Numeral 7 and 8 respectively denote respectively a pay-off reel and a tension reel for the sheet 3 which runs in the direction indicated by the arrow. In this apparatus the grain oriented silicon steel sheet 3 paid off from the pay-off reel 7 passes through a vacuum chamber 1. The portion of the steel sheet 3 directly under the electron beam gun 4 is irradiated by the electron beam 6 which scans the steel sheet 3 linearly in a breadthwise direction substantially perpendicular to the direction of rolling. As a result of the irradiation minute linear thermal strain regions are introduced into the grain oriented silicon steel sheet 3, thus refining the magnetic domain structure, thereby reducing its core loss. The sheet 3 thus treated is then taken up by the tension reel 8.

The particular grain oriented silicon steel sheet employed in the foregoing experiment was obtained by the following process: A hot-rolled steel sheet was prepared which had a composition containing C: 0.065 wt %, Si: 3.38 wt %, Mn: 0.080 wt %, Al: 0.028 wt %, S: 0.030 wt % and N: 0.0068 wt % and the balance substantially Fe. The hot-rolled steel sheet was then uniformly annealed for 3 minutes at 1150° C., followed by quenching. The steel sheet was then warm-rolled at 300° C. until 0.23 mm thick. Subsequently decarburization annealing was conducted in a humid hydrogen atmosphere at 850° C., and an annealing separation agent mainly composed of MgO was applied to the surfaces of the steel sheet. Secondary recrystallization was then effected by raising the temperature from 850° C. to 1150° C. at a rate of 8° C./hour, followed by purifying annealing for 8 hours in a dry hydrogen atmosphere at 1200° C.

Subsequently, an insulating film was applied and baked and then flattening annealing was conducted, whereby the grain oriented silicon steel sheet, as the steel sheet to be employed in the experiment, was prepared. This grain oriented silicon steel sheet had the following magnetic characteristics.

Iron loss ( $W_{17/50}$ ): 0.88 W/kg

Magnetic flux density: ( $B_g$ ): 1.92 T

Samples were prepared by irradiating electron beams under the following test conditions which were combined in various manners so that 162 samples in total were prepared.

Beam acceleration voltage  $V_k$ : 130, 150, 180 kV

Beam current  $I_b$ : 0.6, 0.8, 1.0 mA

Beam diameter  $d$ : 0.20, 0.30 mm

Scanning speed  $v$ : 6, 8, 10 m/sec

Irradiation line spacing  $L$ : 3, 5, 7 mm

Levels of iron loss were measured on all 162 samples. Three-leg core type stacked transformers were fabricated by using about 100 kg of each of the 162 samples, and three-phase voltages were applied to the transformers to activate the transformers for measurements of levels of noise.

The noise (dB) of each transformer was measured by using a sound level meter specified by JIS (Japanese Industrial Standard) 1502 at positions directly above the three legs and at positions spaced 50 cm apart from the respective legs. Then, the mean values of the measured noise levels were calculated as  $dB_i$  ( $i=1$  to 162). The results of the measurement were evaluated by normalizing them to the values at 1.7 T/50 Hz. The noise mea-

surement was conducted by using an A scale as specified by JIS 1502.

Three-leg core stacked transformers also were fabricated by using about 100 kg of each of the 162 samples which were not subjected to the electron beam irradiation, and noise levels were measured while applying three-phase voltages to these transformers. Noise levels were measured at three positions as described above, and the mean values of the measured noise levels were calculated as  $dB'i$  ( $i=1$  to 162). The difference ( $dBi - dB'i$ ) ( $i=1$  to 162) for each sample was determined as the noise characteristic.

FIG. 2 shows the relationship between the iron loss, and the surface energy density  $\alpha$  ( $J/cm^2$ ) of the steel sheet surface as determined by the formula (1) and the surface energy density  $\beta$  ( $J/cm^2$ ) on the beam scanning line as determined by the formula (2).

FIG. 3 shows the relationship between the noise characteristic and the surface energy density  $\alpha$  ( $J/cm^2$ ) of the steel sheet surface and the surface energy density  $\beta$  ( $J/cm^2$ ) on the beam scanning line.

The numbers of points plotted in FIGS. 2 and 3 are smaller than the number of experiments because some of the measured data overlapped.

$$\alpha = (V_k I_b) / (L \cdot v) \quad (1)$$

$$\beta = (V_k I_b) / (d \cdot v) \quad (2)$$

The following criteria were applied for evaluation. More specifically, the criterion for the evaluation of iron loss ( $W_{17/50}$ ) was as shown in Table 1, while the criterion for the evaluation of the noise characteristic was as shown in Table 2.

TABLE 1

| $W_{17/50}$                     | Evaluation | Marks in FIG. 2 | Remarks                                            |
|---------------------------------|------------|-----------------|----------------------------------------------------|
| 0.83 or more                    | Not good   | ●               | Equivalent to conventional products                |
| 0.78 or more but less than 0.83 | Good       | ○               | Product standards graded up by $\frac{1}{2}$ grade |
| Less than 0.78                  | Excellent  | ◎               | Product standards graded up by 1 grade             |

TABLE 2

| Noise Difference $dBi - dB'i$ (dB) | Evaluation | Marks in FIG. 3 | Remarks                            |
|------------------------------------|------------|-----------------|------------------------------------|
| 5 or more                          | Not good   | ●               | No noise suppression effect        |
| 2 or more but less than 5          | Good       | ○               | Noise suppression effect produced  |
| Less than 2                        | Excellent  | ◎               | Remarkable noise prevention effect |

The following will be understood from the foregoing experimental results.

In regard to iron loss, a superior iron loss characteristic is obtained when the surface energy density  $\alpha$  is about  $0.16 J/cm^2$  or more while approximately meeting the condition of  $\alpha \geq 0.6 - 0.06 \beta$ .

It is also understood that an allowable noise characteristic is obtained when a condition of about  $\alpha \geq 0.90 - 0.08 \beta$  is met.

From these results, it is understood that, in order to simultaneously achieve both reduction in iron loss and reduction in noise, it is important that the surface en-

ergy density  $\alpha$  is about  $0.16 J/cm^2$  or more and approximately the condition of the following formula (3) is met.

$$0.6 - 0.06 \beta \leq \alpha \leq 0.9 - 0.08 \beta \quad (3)$$

If one or both of these requirements are not met, either the iron loss or the noise level requirements, or both, are not satisfied.

The method of the present invention offers a remarkable increase of irradiation speed not only over conventional magnetic domain refining methods employing laser beams or plasma but also over known magnetic domain refining methods using electron beams as disclosed in U.S. Pat. No. 4,919,733, so that the speed of treatment of the steel sheet is remarkably increased, thus contributing greatly to increase yield.

For instance, the speed of irradiation employed in the method of the present invention is about 4 times as high as that of the practical example shown in U.S. Pat. No. 4,919,733. In the practical example the surface energy density  $\alpha$  on the steel sheet surface was  $34 J/cm^2$ , while the surface energy density  $\beta$  of the beam scan line was  $0.74 J/cm^2$ . Thus, the surface energy density  $\alpha$  was significantly outside the range of the present invention.

According to the invention superior iron loss characteristic, as well as an improved noise characteristic, is obtained when the surface energy density  $\alpha$  is about  $0.16 J/cm^2$  or more while the approximate condition of the formula (3) mentioned above is met.

We consider that these effects are attributable to the following facts. When a steel sheet is irradiated with an electron beam, tension is generated between adjacent irradiation lines due to thermal strain which is caused by rapid thermal expansion occurring in the irradiated portions. Consequently, magnetic domains are refined to reduce abnormal eddy current loss. However, the thermal expansion causes thermal strain which degrades the noise characteristics. Thus, not only the surface energy density on the beam scan line but also the surface energy density of steel sheet including elements between adjacent irradiation lines is a significant factor which determines iron loss and noise characteristics of the transformer as the product.

Although substantially any practical grain oriented silicon steel sheet composition known heretofore may be employed in the present invention, the following composition and components are preferably employed: C: about 0.01 to 0.10 wt %

This element is effective in uniformly refining the structure both in hot rolling and cold rolling, and also serves in development of Goss orientation. To obtain appreciable effects, the C content should preferably be about 0.01 wt % or more. However, the Goss orientation is disturbed when the C content exceeds about 0.10 wt %. The C content, therefore, should not exceed about 0.10 wt %. Si: about 2.0 to 4.5 wt %

This element effectively contributes to reduction of iron loss by enhancing the specific resistance of the steel sheet. Si content less than about 2.0 wt %, however, causes not only a reduction specific resistance but also random crystal orientation as a result of an  $\alpha$ - $\gamma$  transformation which takes place in the course of final hot annealing which is conducted for the purpose of secondary recrystallization/annealing, thus hampering reduction of iron loss. Conversely, cold rolling characteristics are impaired when the Si content exceeds about 4.5 wt %. The lower and upper limits of the Si content,

therefore, are preferably set to about 2.0 wt % and 4.5 wt %. Mn: about 0.02 to 0.12 wt %

In order to avoid hot embrittlement the Mn content should be at least about 0.02 wt %. Excessive Mn content, however, degrades the magnetic characteristics. The upper limit of the Mn content, therefore, is set to about 0.12 wt %.

Inhibitors suitably employed can be sorted into three types: MnS type, MnSe type and AlN type. When an inhibitor of the MnS type or MnSe type is used, one or both inhibitors selected from the group consisting of S: about 0.005 to 0.06 wt % and Se: about 0.005 to 0.06 wt % is preferably used.

S and Se are elements which can effectively be used as an inhibitor which controls secondary recrystallization in grain oriented silicon steel sheet. For obtaining sufficient inhibition the inhibitor should be present in an amount of at least about 0.005 wt %. The effect of the inhibitor, however, is impaired when its content exceeds about 0.06 wt %. Therefore the lower and upper limits of the content of S or Se are set to about 0.005 wt % and 0.06 wt %, respectively.

When an inhibitor of AlN type is used, both Al: about 0.005 to 0.10 wt % and N: about 0.004 to 0.015 wt % should be present. The contents of Al and N should be determined to fall within the above-mentioned ranges of contents of inhibitor of MnS or MnSe type for the same reasons as stated above.

It is also possible to use other elements than S, Se and Al as the inhibitor, such as Cr, Mo, Cu, Sn, Ge, Sb, Te, Bi and P. Trace amounts of these elements may be used in combination as the inhibitor. More specifically, contents of Cr, Cu and Sn are preferably not less than about 0.01 wt % but not more than about 0.50 wt %, whereas, for Mo, Ge, Sb, Te and Bi, the contents are preferably not less than about 0.005 wt % but not more than about 0.1 wt %. The content of P is preferably not less than about 0.01 wt % but not more than about 0.2 wt %. Each of these inhibitors may be used alone or a plurality of such inhibitors may be used in combination.

The following Examples further illustrate the invention. They are not intended to limit the scope of the invention, which is defined in the appended claims.

#### Example 1

A hot-rolled steel sheet having a composition containing C: 0.063 wt %, Si: 3.40 wt %, Mn: 0.082 wt %, Al: 0.024 wt %, S: 0.023 wt %, Cu: 0.06 wt % and Sn: 0.08 wt % was subjected to a uniformizing annealing conducted for 3 minutes at 1150° C., followed by quenching. Warm rolling was conducted at 300° C., whereby a final cold-rolled sheet of 1000 mm wide and 0.23 mm thick was obtained.

Subsequently, after decarburization annealing in warm hydrogen at 850° C., an anneal separation agent, mainly composed of Al<sub>2</sub>O<sub>3</sub> (80 wt %), MgO (15 wt %) and ZrO<sub>2</sub> (5 wt %), was applied to the surfaces of the steel sheet. Secondary recrystallization was conducted by heating the steel sheet from 850° C. up to 1150° C. at a rate of 10° C./hr, followed by 8-hour purifying annealing at 1200° C. and subsequent flattening annealing for baked insulation coat layer, whereby a grain oriented silicon steel sheet was obtained as the steel sheet to be used in the experiment.

Using this steel sheet a plurality of coils, each being 65 10 tons in weight, were produced.

One of these coils was subjected to irradiation with an electron beam applied within the ranges of irradia-

tion conditions of the invention in the direction perpendicular to the rolling direction by the electron beam irradiation apparatus shown in FIG. 4. At the same time, irradiation with an electron beam was also applied under conditions outside the ranges specified by the invention, thus effecting refining of the magnetic domains. The conditions of irradiation with the electron beam were as follows:

Beam acceleration voltage  $V_k$ : 150 kV

Beam current  $I_b$ : 0.9 mA

Scanning speed  $v$ : 1000 cm/sec

Irradiation line spacing  $L$ : 0.6 cm

Beam diameter  $d$ : 0.02 cm

$\alpha$ : 0.23 J/cm<sup>2</sup>

$\beta$ : 6.8 J/cm<sup>2</sup>

The irradiation apparatus shown in FIG. 4 was materially the same as that shown in FIG. 1. The apparatus employed three electron beam guns 4 arranged in the direction of the sheet breadth at a spacing in the direction of the run of the sheet. This apparatus was of the so-called air-to-air type in which steel sheet 3 was introduced from the exterior of the vacuum chamber 1 through pressure-differential chambers provided in the inlet side of the vacuum chamber 1 and the treated sheet was taken up by a tension reel 8 on the outside of the vacuum chamber 1 through pressure-differential chamber 10 provided on the outlet side of the vacuum chamber 1.

Samples were picked up from several portions on the 30 leading and trailing ends of the coil of the steel sheet produced in accordance with the present invention, and the iron loss ( $W_{17/50}$ ) and the magnetic flux density ( $B_8$ ) were determined for each sample. Mean values of the iron loss and the iron loss and magnetic flux densities at the leading and trailing ends are shown in Table 3.

For the purpose of comparison, mean values of the iron loss ( $W_{17/50}$ ) and magnetic flux density ( $B_8$ ) were measured on the leading and trailing ends of coils produced from the same steel sheets as above but not subjected to irradiation with an electron beam. The results 40 are shown in Table 4.

TABLE 3

| Sampling Position         | Magnetic characteristics of steel sheets Produced by the Method of the Invention (Compared to Table 4) |                                      |                                 |                                                    |
|---------------------------|--------------------------------------------------------------------------------------------------------|--------------------------------------|---------------------------------|----------------------------------------------------|
|                           | Iron Loss $W_{17/50}$ (W/kg)                                                                           | Iron Loss $\Delta W_{17/50}$ (W/kg)* | Magnetic Flux Density $B_8$ (T) | Magnetic Flux Density Difference $\Delta B_8$ (T)* |
|                           | Leading End (Mean Value)                                                                               | 0.785                                | 0.114                           | 1.923                                              |
| Trailing End (Mean Value) | 0.775                                                                                                  | 0.115                                | 1.924                           | -0.002                                             |

\*Difference between values obtained with irradiated steel sheet and steel sheet not irradiated.

TABLE 4

| Sampling Position         | Magnetic characteristics of steel sheets Not Irradiated with Electron Beam |                                 |
|---------------------------|----------------------------------------------------------------------------|---------------------------------|
|                           | Iron Loss $W_{17/50}$ (W/kg)                                               | Magnetic Flux Density $B_8$ (T) |
| Leading End (Mean Value)  | 0.899                                                                      | 1.925                           |
| Trailing End (Mean Value) | 0.890                                                                      | 1.926                           |

Using 5.1 tons of the steel sheet produced in accordance with the present invention, a stacked transformer having three-leg type core was produced and a three-phase voltage was applied to the transformer for mea-

surement of noise generated during the operation of the transformer. The capacity of the transformer was 9000 KVA, while the transformation ratio was 66/6.6 KV.

The measurement of the noise (dB) of the transformer was conducted at positions directly above the these legs and of the core 50 cm spaced apart from the respective legs, by using a sound level meter specified by JIS 1502, and the mean value of the noise levels measured at these three positions was calculated. The measurement of the noise level was conducted by using an A scale as specified in JIS 1502. The results of measurement of noise are shown in Table 5.

By way of comparison, a stacked transformer similar to that shown above was fabricated using a coil made from the same steel sheet which was not subjected to electron beam irradiation. The results of measurement of the noise are shown in Table 6.

TABLE 5

| Characteristics of Stacked Transformer of Invention (Compared to Table 6) |                                                                                                         |            |                                                                            |
|---------------------------------------------------------------------------|---------------------------------------------------------------------------------------------------------|------------|----------------------------------------------------------------------------|
| Iron Loss W <sub>17/50</sub> (W/kg)                                       | Iron Loss Difference From Transformer Made of Non-irradiated Steel Sheet ΔIron Loss, W <sub>17/50</sub> | Noise (dB) | Noise Difference From Transformer Made of Non-irradiated Steel Sheet (ΔdB) |
| 0.933                                                                     | 0.15                                                                                                    | 52         | 1                                                                          |

TABLE 6

| Characteristic of Stacked Transformer Made from Steel Sheet Not Irradiated With Electron Beam |            |
|-----------------------------------------------------------------------------------------------|------------|
| Iron Loss W <sub>17/50</sub> (W/kg)                                                           | Noise (dB) |
| 1.083                                                                                         | 51         |

From Tables 3 and 5, it will be understood that both iron loss and noise characteristic are remarkably improved according to the present invention which employs electron beam irradiation under the specified conditions.

According to the aforesaid criteria of evaluation, the iron loss of the steel sheet produced in accordance with the method of the present invention is "Good". The noise characteristic of the stacked transformer of the present invention was "Excellent".

### Example 2

Refining of magnetic domains on a grain oriented silicon steel sheet the same as that in Example 1 was effected by electron beam irradiation in the same manner as Example 1 under the following conditions which fall within the range of the present invention. The iron loss of the steel sheet obtained through this treatment, as well as the noise of the stacked transformer, was measured by the same method as Example 1. The results of the measurement are shown in Tables 7 and 8.

From these Tables it will be understood that both the iron loss and the noise characteristics were significantly improved as a result of the electron beam irradiation executed under the conditions:

Beam acceleration voltage V<sub>k</sub>: 200 kV  
 Beam current I<sub>b</sub>: 0.4 mA  
 Scanning speed v: 500 cm/s  
 Irradiation line spacing L: 0.4 cm  
 Beam diameter d: 0.03 cm  
 $\alpha$ : 0.4 J/cm<sup>2</sup>  
 $\beta$ : 5.3 J/cm<sup>2</sup>

TABLE 7

| Magnetic Characteristics of Steel Sheet of Invention (Compared to Table 4) |                                     |                                       |                                          |                                                       |
|----------------------------------------------------------------------------|-------------------------------------|---------------------------------------|------------------------------------------|-------------------------------------------------------|
| Sampling Position                                                          | Iron Loss W <sub>17/50</sub> (W/kg) | Iron Loss ΔW <sub>17/50</sub> (W/kg)* | Magnetic Flux Density B <sub>8</sub> (T) | Magnetic Flux Density Difference ΔB <sub>8</sub> (T)* |
| Leading End (Mean Value)                                                   | 0.779                               | 0.120                                 | 1.922                                    | -0.003                                                |
| Trailing End (Mean Value)                                                  | 0.789                               | 0.121                                 | 1.923                                    | -0.002                                                |

\*Difference between values obtained with irradiated steel sheet and steel sheet not irradiated.

TABLE 8

| Characteristics of Stacked Transformer of Invention (Compared to Table 6) |                                                                                                         |            |                                                                            |
|---------------------------------------------------------------------------|---------------------------------------------------------------------------------------------------------|------------|----------------------------------------------------------------------------|
| Iron Loss W <sub>17/50</sub> (W/kg)                                       | Iron Loss Difference From Transformer Made of Non-irradiated Steel Sheet ΔIron Loss, W <sub>17/50</sub> | Noise (dB) | Noise Difference From Transformer Made of Non-irradiated Steel Sheet (ΔdB) |
| 0.929                                                                     | 0.154                                                                                                   | 53         | 2                                                                          |

### Comparative Example 1

A magnetic domain refining treatment was conducted on a coil made of the same grain oriented silicon steel sheet same as that of Example 1, by applying an electron beam under the following conditions which did not satisfy the requirement of formula (3) of the present invention. The iron loss of the steel sheet thus obtained, as well as the noise of the stacked transformer, was measured by the same method as Example 1. The results of the measurement are shown in Tables 9 and 10.

From Tables 9 and 10 it will be understood that the noise characteristic of the transformer was inferior, although good iron loss characteristics were obtained, due to the fact that the conditions of irradiation with the electron beam did not meet the requirement of formula (3).

Beam acceleration voltage V<sub>k</sub>: 100 kV  
 Beam current I<sub>b</sub>: 1.0 mA  
 Scanning speed v: 500 cm/s  
 Irradiation line spacing L: 0.6 cm  
 Beam diameter d: 0.02 cm  
 $\alpha$ : 0.33 J/cm<sup>2</sup>  
 $\beta$ : 10 J/cm<sup>2</sup>

TABLE 9

| Magnetic Characteristics of Steel Sheet of Comparative Example 1 (Compared to Table 4) |                                     |                                       |                                          |                                                       |
|----------------------------------------------------------------------------------------|-------------------------------------|---------------------------------------|------------------------------------------|-------------------------------------------------------|
| Sampling Position                                                                      | Iron Loss W <sub>17/50</sub> (W/kg) | Iron Loss ΔW <sub>17/50</sub> (W/kg)* | Magnetic Flux Density B <sub>8</sub> (T) | Magnetic Flux Density Difference ΔB <sub>8</sub> (T)* |
| Leading End (Mean Value)                                                               | 0.775                               | 0.124                                 | 1.922                                    | -0.003                                                |
| Trailing End (Mean Value)                                                              | 0.774                               | 0.136                                 | 1.921                                    | -0.005                                                |

\*Difference between values obtained with irradiated steel sheet and steel sheet not irradiated.

TABLE 10

| Characteristics of Stacked Transformer of Comparative Example 1 (Compared to Table 6) |                  |  |
|---------------------------------------------------------------------------------------|------------------|--|
| Iron Loss Difference From Trans-                                                      | Noise Difference |  |
|                                                                                       |                  |  |

TABLE 10-continued

| Iron Loss<br>W <sub>17/50</sub><br>(W/kg) | former Made of Non-<br>irradiated Steel<br>Sheet ΔIron Loss,<br>W <sub>17/50</sub> | Noise<br>(dB) | From Transformer<br>Made of Non-<br>irradiated Steel<br>Sheet (ΔdB) |
|-------------------------------------------|------------------------------------------------------------------------------------|---------------|---------------------------------------------------------------------|
| 0.930                                     | 0.153                                                                              | 60            | 9                                                                   |

## Comparative Example 2

A magnetic domain refining treatment was conducted on a coil made of the same grain oriented silicon steel sheet same as that of Example 1, by applying an electron beam under the following conditions which did not satisfy the requirement of formula (3) in accordance with the present invention. The iron loss of the steel sheet thus obtained, as well as the noise of the stacked transformer, was measured by the same method as Example 1. The results of the measurement are shown in Tables 11 and 12.

From Tables 11 and 12 it will be understood that the iron loss characteristic was inferior, although a good noise characteristic of the transformer was obtained, due to the fact that the conditions of irradiation with the electron beam did not meet the requirements of formula (3):

Beam acceleration voltage  $V_k$ : 150 kV

Beam current  $I_b$ : 0.8 mA

Scanning speed  $v$ : 900 cm/s

Irradiation line spacing  $L$ : 0.7 cm

Beam diameter  $d$ : 0.03 cm

$\alpha$ : 0.19 J/cm<sup>2</sup>

$\beta$ : 4.4 J/cm<sup>2</sup>

TABLE 11

Magnetic Characteristics of Steel Sheet of Comparative Example 2 (Compared to Table 4)

| Sampling Position         | Iron Loss<br>W <sub>17/50</sub><br>(W/kg) | Iron Loss<br>ΔW <sub>17/50</sub><br>(W/kg)* | Magnetic Flux Density<br>$B_8$ (T) | Magnetic Flux Density Difference<br>Δ $B_8$ (T)* |
|---------------------------|-------------------------------------------|---------------------------------------------|------------------------------------|--------------------------------------------------|
| Leading End (Mean Value)  | 0.862                                     | 0.037                                       | 1.925                              | 0                                                |
| Trailing End (Mean Value) | 0.860                                     | 0.050                                       | 1.926                              | 0                                                |

\*Difference between values obtained with irradiated steel sheet and steel sheet not irradiated.

TABLE 12

Characteristics of Stacked Transformer of Comparative Example 2 (Compared to Table 6)

| Iron Loss<br>W <sub>17/50</sub><br>(W/kg) | Iron Loss Difference From Transformer Made of Non-irradiated Steel Sheet ΔIron Loss,<br>W <sub>17/50</sub> | Noise<br>(dB) | Noise Difference From Transformer Made of Non-irradiated Steel Sheet (ΔdB) |
|-------------------------------------------|------------------------------------------------------------------------------------------------------------|---------------|----------------------------------------------------------------------------|
| 1.04                                      | 0.043                                                                                                      | 52            | 1                                                                          |

As will be understood from the foregoing description, according to the present invention, it is possible to obtain a low-iron-loss grain oriented silicon steel sheet for use as the material of a stacked core transformer, the steel sheet simultaneously exhibiting both superior iron characteristics and excellent noise characteristics in the stacked transformer, by virtue of the fact that irradiation with the electron beam is executed at specified levels of energy density of the beam scan line and of surface energy density. In addition, the present inven-

tion offers remarkable improvements of production efficiency.

What is claimed is:

1. A method of producing a grain oriented silicon steel sheet having reduced iron loss and which, when used as a material in a stacked transformer, makes it possible to obtain a noise difference (dB<sub>i</sub> - dB'<sub>i</sub>) less than 5 dB, said method comprising:

preparing a finish-annealed grain oriented silicon steel sheet;

irradiating the surface of said grain oriented silicon steel sheet with an electron beam directed along scan paths which cross the rolling direction of said steel sheet,

said irradiation being applied to said sheet at a scanning speed  $v$ (cm/s) and a spacing  $L$ (cm) in the rolling direction, with an electron beam having a beam diameter  $d$ (cm) generated by a current  $I_b$  (mA) and an acceleration voltage  $V_k$  (kV);

wherein said beam is applied with a surface energy density  $\alpha$  (J/cm<sup>2</sup>) on the surface of said steel sheet as determined by the following formula (1), and is about 0.16 J/cm<sup>2</sup> or more,

and wherein said surface energy density  $\alpha$  (J/cm<sup>2</sup>) and a surface energy density  $\beta$  (J/cm<sup>2</sup>) on the scan paths meet the approximate condition of the following formula (3):

$$\alpha = (V_k I_b) / (L \cdot v) \quad (1)$$

$$\beta = (V_k I_b) / (d \cdot v) \quad (2)$$

$$0.6 - 0.06\beta \leq \alpha \leq 0.90 - 0.08\beta \quad (3)$$

2. The method defined in claim 1 wherein the steel sheet has a composition of about:

C: 0.01-0.10% by weight

Si: 2.0-4.5% by weight

Mn: 0.02-0.12% by weight

and inhibitors and incidental impurities, and the balance Fe.

3. A stacked transformer made of a grain oriented silicon steel sheet and having a noise difference (dB<sub>i</sub> - dB'<sub>i</sub>) less than 5 dB, said sheet capable of being produced by a method which comprises:

preparing a finish-annealed grain oriented silicon steel sheet;

irradiating the surface of said grain oriented silicon steel sheet with an electron beam directed along scan paths which cross the rolling direction of said steel sheet,

said irradiating having been applied to said sheet at a scanning speed  $v$ (cm/s) and a spacing  $L$ (cm) in the rolling direction, with an electron beam having a beam diameter  $d$ (cm) generated by a current  $I_b$  (mA) and an acceleration voltage  $V_k$  (kV);

wherein said beam has been applied with a surface energy density  $\alpha$  (J/cm<sup>2</sup>) on the surface of said steel sheet as determined by the following formula (1), and is about 0.16 J/cm<sup>2</sup> or more,

and wherein said surface energy density  $\alpha$  (J/cm<sup>2</sup>) and a surface energy density  $\beta$  (J/cm<sup>2</sup>) on the scan paths meet the approximate condition of the following formula (3):

$$\alpha = (V_k I_b) / (L \cdot v) \quad (1)$$

$$\beta = (V_k I_b) / (d \cdot v) \quad (2)$$

0.6-0.06 $\beta$   $\leq$   $\alpha$   $\leq$  0.90-0.08 $\beta$ 

4. The slackened transformer defined in claim 3 wherein the steel sheet has a composition of about:

C: 0.01-0.10% by weight

Si: 2.0-4.5% by weight

Mn: 0.02-0.12% by weight

and inhibitors and incidental impurities, and the balance Fe.

5. A stacked transformer having a noise difference (dB<sub>i</sub>-dB'<sub>i</sub>) less than 5 dB, said transformer comprising finish-annealed grain oriented silicon steel sheet having reduced iron loss, said sheet having been irradiated by an electron beam having a diameter d (cm) generated by a current I<sub>b</sub> (mA) and an acceleration voltage V<sub>k</sub> (kV), said beam having been applied to a surface of said sheet at a scanning speed v (cm/s) in scan paths spaced by distance L (cm) to provide a surface energy density  $\alpha$  (J/cm<sup>2</sup>) on said surface and a path energy density  $\beta$  (J/cm<sup>2</sup>) on each of said paths, said surface energy density  $\alpha$  and path energy density  $\beta$  satisfying formulas (1)-(3):

$$\alpha = (V_k I_b) / (L \cdot v) \quad (1)$$

$$\beta = (V_k I_b) / (d \cdot v) \quad (2)$$

0.6-0.06 $\beta$   $\leq$   $\alpha$   $\leq$  0.90-0.08 $\beta$ 

(3).

6. The stacked transformer of claim 5 wherein said sheet comprises about 0.01-0.10 wt % of C, 2.0-4.5 wt % of Si, and 0.02-0.12 wt % of Mn.

7. A stacked transformer having a noise difference (dB<sub>i</sub>-dB'<sub>i</sub>) less than 5 dB, said transformer comprising finish-annealed grain oriented silicon steel sheet with reduced iron loss, said sheet being capable of being produced by a method comprising the steps of:

10 preparing said finish-annealed grain oriented silicon steel sheet; and  
 irradiating the surface of said sheet with an electron beam directed along scan paths which cross the rolling direction of said steel sheet, said electron beam being applied to said sheet at a scanning speed v (cm/s) and a spacing L (cm) in the rolling direction, said electron beam being generated by a current I<sub>b</sub> (mA) and an acceleration voltage V<sub>k</sub> (kV) and having a beam diameter d (cm), wherein said beam is applied with a surface density  $\alpha$  (J/cm<sup>2</sup>) of at least about 0.16 J/cm<sup>2</sup> on the surface of said sheet and a surface density  $\beta$  (J/cm<sup>2</sup>) on said scan paths according to the following formulas:

$$\alpha = (V_k I_b) / (L \cdot v);$$

$$\beta = (V_k I_b) / (d \cdot v); \text{ and}$$

0.6-0.06 $\beta$   $\leq$   $\alpha$   $\leq$  0.90-0.08 $\beta$ .

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999

UNITED STATES PATENT AND TRADEMARK OFFICE  
**CERTIFICATE OF CORRECTION**

PATENT NO. : 5,411,604

DATED : May 2, 1995

INVENTOR(S) : Yukio Inokuti, Kazuhiro Suzuki and Eiji Hina

It is certified that error appears in the above-identified patent and that said Letters Patent is hereby corrected as shown below:

In Column 3, line 49, please change "DRAWING" to --DRAWINGS--.

In Column 5, line 65, please change "≥" to --≤--.

In Column 7, line 48, please change "Ai" to --Al--.

In Column 13, line 3, please change "slacked" to --stacked--.

Signed and Sealed this

Eighteenth Day of July, 1995

Attest:



BRUCE LEHMAN

Attesting Officer

Commissioner of Patents and Trademarks